# EUROPEAN PATENT SPECIFICATION

(11) **EP 1 320 640 B1**
(45) Date of publication and mention of the grant of the patent: **04.03.2009**
(21) Application number: 01960785.2
(22) Date of filing: 09.08.2001
(51) Int. Cl.: D21C 1/02, D21B 1/02

(54) **STEAMING PROCESS**
DÄMPFUNGSVERFAHREN
PROCEDE DE TRAITEMENT A LA VAPEUR

(30) Priority: 14.08.2000 FI 20001787
(43) Date of publication of application: 25.06.2003
(73) Proprietor: Fortum OYJ, 02150 Espoo (FI)
(72) Inventor: REPKA, Mika, FIN-00920 Helsinki (FI)
(74) Representative: Kurra, Sirpa Eliina
(86) International application number: PCT/FI2001/000703
(87) International publication number: WO 2002/014599

(56) References cited:
- SE-B- 420 224
- US-A- 3 801 431
- US-A- 4 012 279
- DATABASE PAPERCHEM [Online] KROTOV V.S. ET AL.: 'Increasing the effectiveness of the Pandia digester', XP002963125 Retrieved from Dialog, accession no. 00208867 Database accession no. AB5509836 & BUMAZH. PROM. no. 6, June 1984, pages 20 - 24

## Description

The present invention relates to a method of steaming lignocellulosic material to change the structure of the material and to impregnate the lignocellulosic material to be pulped with delignifying chemicals. In the method, lignocellulosic material is steamed before it is impregnated with a delignifying chemical solution. Lignocellulosic material means in this connection all material of plant origin used as raw material in a chemical pulp cook, such as wood, straw, grass, bagasse, etc. The lignocellulosic material used in the method is, when needed, in a form cut in a conventional manner for delignification, for example, wood material as chips or sawdust.

In this connection, pulping refers to the pulping of lignocellulosic material, which includes some degree of delignification of the lignocellulosic material which takes place by means of chemicals and heat. The delignification accomplished with chemicals and heat may be supplemented with mechanical defibring to achieve the desired degree of defibring.

By delignifying chemicals are meant in this connection all chemicals commonly used for the purpose in question, which chemicals are absorbed into lignocellulosic material and which dissolve or soften the lignin contained in the material and by which delignification is accomplished at a temperature higher than ambient temperature. As examples, sulphate and sulphite pulp cooking liquors may be mentioned.

The reactions of the lignin contained in fibre material with dissolving and/or softening chemicals take place in the desired manner only if the chemicals have penetrated uniformly and thoroughly into the material which is being pulped. The absorption of chemicals is influenced by two mechanisms, penetration and diffusion. In natural penetration, cooking chemical liquor penetrates into fibre material through its capillary structure by the action of capillary forces. The penetration process may be assisted by providing a pressure difference across the capillary structure.

The speed and thorough accomplishment of the penetration process is greatly dependent on the air which is contained in fibre material and which should be removed before treating the material with delignifying chemicals. One method used is the deaeration of fibre material by steaming. During steaming, the air contained in fibre material expands through heating, and partly escapes from the pore spaces of fibre material. The steam used in the treatment penetrates, in turn, into the pore spaces of fibre material where it contributes to the exit of air from the pores of fibre material through condensation and vaporisation processes.

Prior art steaming processes have used saturated steam. The upper limit of the temperature of steam has been considered to be 120 -126°C and, at temperatures higher than this, the hydrolysis of fibre materials has been considered to accelerate to a detrimental extent. The condensation of lignin at higher temperatures has also been considered to be a problem.

US 3,801,431 discloses a method for heating of wooden chips in preparation for the production of pulp by digestion. Pretreatment is carried out in three successive pressure vessels. The temperature of the steam in each pressure vessel corresponds to the temperature of saturated steam at the pressure prevailing in the vessel.

US 3,619,348 discloses a method in which a downwardly moving column of cellulosic material is contacted in a steaming zone with a countercurrent flow of steam at atmospheric pressure and at a temperature not exceeding 120 °C to expel air from the material without causing discoloration thereof, after which the steamed material is preimpregnated with a cold liquor in a sealed zone.

Steaming of lignocellulose containing fibre material in accordance with the prior art with saturated steam inevitably leads to an increase in the moisture content of the fibre material, because substantially the entire steam amount used in steaming condenses on the fibre material and penetrates into its structures. The condensation energy of steam correspondingly increases the temperature of the fibre material that is being treated. On the other hand, the steam condensing on the surface layers of the fibre material prevents escape of air.

In accordance with the basic idea of the invention, steaming of lignocellulose based fibre material is carried out in a steam atmosphere under superheated conditions, and the lignocellulosic material is maintained substantially at the steaming pressure up to at least an impregnation stage. The steaming is advantageously accomplished by passing superheated steam into contact with the fibre material. Also other means of introducing energy, such as indirect heating or an inert energy carrier (such as fluidised bed material), are feasible enabling a steam atmosphere under superheated conditions to be maintained during steaming.

When using superheated steam passed to the fibre material, the inlet and the final temperatures of steam are determined according to the material of the fibre material being processed. In treatment tests of bio-mass, the temperature of incoming steam has varied in a range of from 270 °C to 350 °C and the temperature of exiting steam has been determined according to saturated steam pressure corresponding to operating pressure (max. 23 bar(abs)) such that its superheating has been by about 15 °C - 25 °C higher than the saturated state.

Superheated steam has a strong effect on the fibre material to be treated. Firstly, superheated steam binds into itself water from the fibre material and, secondly, causes an increase in the temperature of the fibre material. The water present in the fibre material vaporises, passes to the surface of the material and exits with superheated steam out of connection with the fibre material. At the same time, vaporising water drives the air present in the fibre structure out of the fibre. An essential factor is also that the vaporising water most evidently opens the capillary and pore structure of the fibre.

From the viewpoint of carrying out of the invention it is essential that the fibre is maintained under conditions where this open space of capillaries and pores is preserved as far as possible into the absorption process of delignifying chemicals. In this respect, the residual moisture of fibre material and the ambient atmosphere are crucial.

Attempts are made to maintain the fibre material in such a state that there is residual moisture at least in a vapour state in its structure. The best situation is achieved if there is moisture in such an amount and in such a state that it still tends to vaporise and force its way out of the structure. This assures that the pore structure remains open. On the other hand, the moisture vaporising in the fibre structure binds heat, which prevents the temperature of the fibre material from rising so high that detrimental degradation and condensation reactions of the fibre material are initiated. In respect of residual moisture, the crucial factor is the time during which the fibre material is in contact with superheated steam, in addition to the superheating degree of the ambient steam atmosphere. The state of the ambient atmosphere is in turn determined by the pressure prevailing in it.

When fibre material which has been steamed and the pore structure of which is in an open state (containing vaporised moisture and being at least at a pressure of saturated steam corresponding to ambient temperature) is brought into contact with a solution containing delignifying chemicals, the solution will penetrate into the fibre structure replacing the moisture which has escaped from there. The penetration of the solution into the fibre structure can be promoted by creating a situation where the moisture present in the fibre structure is condensed, whereby a corresponding underpressure is produced between the pores of the fibre structure and the environment. This situation can be created, for example, by using a delignifying chemical solution that is slightly colder than the saturated state of the fibre structure.

Said arrangement has been found to allow rapid absorption of delignifying solutions uniformly through the entire fibre material. The arrangement also makes it possible that the impregnated fibre material is substantially at delignification temperature after impregnation. The detrimental reactions of fibre raw material and delignifying chemicals associated with slow absorption and with slow heating to delignification temperature can thus be eliminated.

In the steaming of lignocellulosic material accomplished by superheated steam, the contact time between the material and steam is substantially short, of course, depending on the particle size of the material. For example, in the case of fine wood raw material (classified with the definition "sawdust", the particle size being about 3-5 mm) an appropriate dwell time is of the order of seconds.

The steaming stage of the invention can be accomplished in a processing apparatus of the so-called flash type in which fine lignocellulosic material is supplied to be carried with a superheated steam flow, and is separated from this flow after an appropriate dwell time. The apparatus is illustrated in the accompanying drawing, in which
Figure 1 shows one embodiment of the steaming and impregnation apparatus in accordance with the invention, and
Figure 2 shows an apparatus used for a similar purpose, as an alternative embodiment in respect of the impregnation apparatus.

In the embodiments shown in the drawing figures the steaming apparatus comprises a steam flow circulation 1 which includes a fan 3 maintaining the circulation, a superheating device 2 (boiler), a steaming stage 4 situated after the superheating device and having at its lower end feed devices 5 for feeding lignocellulosic material, a steam separator 6, excess steam exhaust 7, as well as a seal type feeder 8 for lignocellulosic material. When needed, the apparatus also includes a return circulation 10 for steamed lignocellulosic material.

In the embodiment shown in Fig. 1, the steamed lignocellulosic material is shown to be fed through the seal type feeder 8 into an impregnation device 11, into which a solution containing delignifying chemicals is fed from a tank 9. The impregnation device may have a structure known in the art. Inside it there is usually a screw feeder with a gentle pitch, which conveys lignocellulose containing fibre material through the impregnation device along an obliquely upwards rising path. In the impregnation device, the delignifying solution is usually maintained at a level that extends to about half the length of the impregnation device. Impregnation takes place in the lower part of the device and discharge of excess solution takes place in the upper part by draining. The excess solution can be passed into the solution tank 9, possibly monitored in respect of the chemical content.

At the discharge end of the impregnation device 11 there is advantageously also a seal type feeder 12, by means of which an independently adjustable pressure can be maintained in the impregnation device 11. The lignocellulosic fibre material is fed from the seal type feeder 12 to a delignification vessel 13 proper, in which delignification reactions are performed to the desired delignification degree. In the delignification vessel 13, a suitable pressure and a corresponding temperature of saturated steam are maintained at which delignification reactions have been found to occur most advantageously from the point of view of fibre material. Temperature can be maintained, for example, in a known manner by means of a liquid circulation provided with heating 15.

The impregnation after steaming can be alternatively accomplished by operating as shown in Fig. 2. In this embodiment, a press can serve as the seal type feeder 8. A solution containing delignifying chemicals can be fed into the fibre material in connection with the press and excess solution can be squeezed out in the press. After that, the impregnated fibre material is passed to the delignification vessel 13, in which the fibre material is/is maintained at delignification temperature in the ambient steam phase. The temperature is maintained by passing direct steam into the vessel from a conduit 16. Alternatively, the temperature can be maintained by indirect heat transfer by means of steam passed from the conduit 16. This apparatus arrangement allows the liquid volume of the process to be minimised.

The fibre material is passed from the delignification vessel 13 through a seal type feeder 14 to possible mechanical defibring, and further to conventional washing and bleaching stages.

The arrangements shown in Figs. 1 and 2 make it possible to use different conditions in different process stages. From the point of view of the total flow of the process it is advantageous that the fibre material is maintained throughout the entire process substantially at a pressure that corresponds to the pressure of the saturated steam of the temperature used in the delignification stage. As a variant of this operation model, it is also possible to operate so that the pressure drops slightly during transition from steaming to impregnation and further during transition from impregnation to the delignification stage. Also other alternatives of pressure and corresponding temperature conditions are feasible when carrying out the invention taking into account the fibre material (the source of material as such, the particle size, moisture content), the chemicals used and the desired delignification degree.

The moisture escaping from the lignocellulosic material which is in contact with superheated steam in the steaming stage 4 is carried with steam into the separator device 6, from which excess circulation steam is discharged through the conduit 7. The energy level of this steam is high, and it can be utilised in later stages of the pulping process, for example, in heating delignifying chemicals, in regeneration stages of the chemicals circulation, in bleaching, in washing, etc. Control of the exhaust steam 7 can also be used for regulating the heating stage 2 of the superheating circulation so that there should prevail an inert gas state in the circulation 1.

## Claims

1. A method for impregnating lignocellulosic material to be pulped with delignifying chemicals before a delignification stage, in which method the lignocellulosic material is treated in a steam atmosphere, and the steamed lignocellulosic material is impregnated with the delignifying chemicals, **characterised in that** the treatment of the lignocellulosic material is carried out in a steam atmosphere under superheated conditions, which superheated state is maintained throughout the treatment, and that the lignocellulosic material is maintained substantially at the pressure of the steaming process up to at least the impregnation stage.

2. A method according to claim 1, **characterised in that** the steaming process is carried out substantially at the pressure of the delignification stage.

3. A method according to claim 2, **characterised in that** the impregnation with the delignifying chemicals is carried out substantially at the pressure of the delignification stage.

4. A method according to claim 1, 2 or 3, **characterised in that** the steamed lignocellulosic material is impregnated with the delignifying chemicals while they are substantially at the temperature of the delignification stage.

5. A method according to claim 1, 2 or 3, **characterised in that** the steamed lignocellulosic material is impregnated with delignifying chemicals while they are at a temperature lower than the delignification temperature.

## Patentansprüche

1. Verfahren zum Imprägnieren von aufzuschließenden Lignocellulose-Material mit delignifizierenden Chemikalien vor einem Delignifizierungsschritt, wobei in dem Verfahren das Lignocellulose-Material in einer Dampfatmosphäre behandelt wird und das dampfbehandelte Lignocellulose-Material mit den delignifizierenden Chemikalien imprägniert wird,
**dadurch gekennzeichnet, daß** die Behandlung des Lignocellulose-Materials in einer Dampfatmosphäre unter überhitzten Bedingungen durchgeführt wird, wobei der überhitzte Zustand während der gesamten Behandlung aufrechterhalten wird, und **dadurch**, daß zumindest bis zu dem Imprägnierungsschritt das Lignocellulose-Material im wesentlichen auf dem Druck des Dampfbehandlungsschritts gehalten wird.

2. Verfahren nach Anspruch 1, **dadurch gekennzeichnet, daß** der Dampfbehandlungsprozeß im Wesentlichen bei dem Druck des Delignifizierungsschritts durchgeführt wird.

3. Verfahren nach Anspruch 2, **dadurch gekennzeichnet, daß** die Imprägnierung mit den delignifizierenden Chemikalien im Wesentlichen bei dem Druck des Delignifizierungsschritts durchgeführt wird.

4. Verfahren nach Anspruch 1, 2 oder 3, **dadurch gekennzeichnet, daß** das dampfbehandelte Lignocellulose-Material mit den delignifizierenden Chemikalien imprägniert wird, während sie im wesentlichen bei der Temperatur des Delignifizierungsschritts sind.

5. Verfahren nach Anspruch 1, 2 oder 3, **dadurch gekennzeichnet, daß** das dampfbehandelte Lignocellulose-Material mit den delignifizierenden Chemikalien imprägniert wird, während sie bei einer Temperatur unterhalb der Delignifizierungstemperatur sind.

## Revendications

1. Procédé d'imprégnation d'une matière lignocellulosique à réduire en pâte avec des produits chimiques de délignification avant un stade de délignification, dans lequel la matière lignocellulosique est traitée dans une atmosphère de vapeur d'eau, et la matière lignocellulosique traitée à la vapeur d'eau est imprégnée avec les produits chimiques de délignification, **caractérisé en ce que** le traitement de la matière lignocellulosique est réalisé dans une atmosphère de vapeur d'eau dans des conditions surchauffées, l'état surchauffé étant maintenu tout au long du traitement, et **en ce que** la matière lignocellulosique est maintenue sensiblement à la pression du procédé de traitement à la vapeur d'eau au moins jusqu'au stade d'imprégnation.

2. Procédé selon la revendication 1, **caractérisé en ce que** le procédé de traitement à la vapeur d'eau est réalisé sensiblement à la pression du stade de délignification.

3. Procédé selon la revendication 2, **caractérisé en ce que** l'imprégnation avec les produits chimiques de délignification est réalisée sensiblement à la pression du stade de délignification.

4. Procédé selon la revendication 1, 2 ou 3, **caractérisé en ce que** la matière lignocellulosique traitée à la vapeur d'eau est imprégnée avec les produits chimiques de délignification pendant qu'ils sont sensiblement à la température du stade de délignification.

5. Procédé selon la revendication 1, 2 ou 3, **caractérisé en ce que** la matière lignocellulosique traitée à la vapeur d'eau est imprégnée avec des produits chimiques de délignification pendant qu'ils sont à une température plus basse que la température de délignification.
